

## UNITED STATES PATENT OFFICE

2,361,352

## LUBRICATING OIL COMPOSITION

Ferdinand P. Otto, Woodbury, N. J., assignor to  
Socony-Vacuum Oil Company, Incorporated,  
New York, N. Y., a corporation of New York

No Drawing. Application December 11, 1941,  
Serial No. 422,518

13 Claims. (Cl. 252—48)

This invention has to do with the treatment of hydrocarbon products such as mineral oils to improve their characteristics, and more specifically to the addition to petroleum lubricating oils of characterizing agents which improve their ability to resist the deteriorating effect of oxidation and their ability to lubricate bearing surfaces which are subjected to extreme pressures such as are now commonly encountered in hypoid gears and the like.

Moderately refined oils, such as motor oils and other moderately refined lubricating oils normally used under conditions of exposure to oxidation in the presence of metals, oxidize to sludge and/or acidic oxidation products normally corrosive to the metals which they encounter in use, as, for example, bearing metals in automotive use. It has now been found that stabilization of these oils against such oxidation effects may be conveniently accomplished by addition to the oils of certain materials which substantially retard the oxidation of the oils, whether or not metal is present, or by the addition of certain other materials which apparently have the ability to inhibit the catalytic effect of metals in promoting oxidation reactions and thus prevent the formation of sludge and/or acidic constituents and the like under normal conditions of use and achieve an equally good practical result, although materials of the latter class may be incapable of inhibiting oxidation of oils in the absence of metals. This invention has to do with stabilizing reaction products which appear to be of this latter class, not heretofore known to be effective for this purpose, and with oils stabilized by the use of these reaction products.

Recent changes in automotive engine design, tending toward higher bearing pressures, higher rotative speeds, higher engine temperatures, etc., have been concurrent with marked advances in methods of refining lubricant oils for automotive use. The demand for oils having lesser changes in viscosity with temperature change, that is, higher viscosity index, commonly referred to as V. I., has been met by refining lubricants intended for motor oils by certain solvent refining or solvent extraction processes. Certain liquid reagents possess solvent power for hydrocarbons of various types; as, for example, dichlorodimethyl ether, cresylic acid, phenol, chloraniline, chlorophenol, phenetidine, benzyl alcohol, nitrobenzene, benzonitrile, furfural, aniline, benzylacetate, liquid sulphur dioxide, mixtures of liquid sulphur dioxide or aniline with benzol, and the like. Those solvent refining processes are designed to

- concentrate in the desired lubricant fraction those compounds of a "paraffinic" nature possessed of the ability to suffer only a small change of viscosity, with changes of temperature, and to reject the compounds of "naphthenic" nature which do suffer such change of viscosity to such a marked degree. These refining processes have provided a supply of an oil of quite desirable general characteristics definitely far superior to 10 any oil previously produced from mixed base or asphaltic crudes, and superior to a like, though lesser, degree over oils previously produced from paraffin base crudes.
- It has been found that the solvent refined 15 motor oils referred to above are definitely corrosive to the newer bearing metals referred to above under normal conditions of automotive use, due to oxidation during use, sometimes resulting in bearing failure after only a few thousand 20 miles of normal driving. It is further known that the same reaction, that is, corrosion of alloy-bearing metals such as cadmium-silver, also occurs in good paraffinic base oils which have not been subjected to solvent refining. The higher 25 the V. I. of the lubricating oil, the more pronounced is the tendency to corrosion of the kind referred to above. Generally speaking, the problem is encountered in oils having a V. I. of 75 or higher, and becomes pronounced in oils having a V. I. of 80 to 85 or higher, and very pronounced in oils of 100 V. I. or higher.
- Furthermore, the present trend in automotive 30 design toward lower body styles, rapid acceleration, and the use of hypoid gears has increased the unit loadings on rear axles. In some cases the unit pressures encountered become great enough to rupture the oil film of ordinary mineral oil lubricants, with consequent metal to metal contact. In other lines of power transmission and the like, there is a similar tendency 35 toward the use of high unit pressures of a degree which are near or beyond the limit at which mineral oils, alone, will maintain effective lubrication. The present invention is, therefore, specifically concerned with the production of lubricants capable of withstanding the high unit loadings which occur in such instances. Such lubricants are generally referred to as extreme pressure 40 agents.
- 50 Lubricants of the extreme pressure type are normally produced by adding to a hydrocarbon lubricating oil a small amount of some characterizing substance which enables it to maintain a lubricant film unruptured under conditions which would cause the breakdown of a film formed of

oil alone. Such additive substances are spoken of as E. P. (extreme pressure) bases, or E. P. ingredients. Many commonly used E. P. bases are composed of sulphur dissolved in mineral oil, sulphurized vegetable or animal oils, chlorinated compounds, metallic soaps, and the like. This invention is specifically concerned with the use, as E. P. characterizing ingredients, of reaction products new and novel for the purpose, and not hitherto so used or known to be useful for this purpose.

It is an object of this invention to provide an extreme pressure lubricant, together with a base for use in compounding same, which lubricant is superior to lubricants of this class heretofore commonly known, particularly in load-carrying capacity, stability, and maintenance of extreme pressure lubricating properties under sustained conditions of high loading. It is an object of this invention to prepare novel and valuable ingredients and to combine them with hydrocarbon lubricant oils to produce lubricants having high load bearing capacities, to prepare such ingredients which have good characteristics of stability, and which are less corrosive than ordinary extreme pressure ingredients. Further objects are the provision of methods of preparing lubricants containing these novel characterizing ingredients and methods of lubrication making use of the lubricants so produced.

It is an important object of this invention to provide means for satisfactorily inhibiting or preventing corrosion from taking place to a serious degree particularly in oils of relatively high viscosity index. It is also an object of this invention to provide a substantially non-corrosive motor oil of high V. I. Still another object of the invention is to provide an additive reagent or ingredient capable of inhibiting the corrosive properties of these oils. The production of solvent refined oils of low corrosive properties under conditions of automotive use is a major object of this invention, as well as the method of production of such oils which combine a relatively high viscosity index with a relatively low tendency to produce such corrosion.

A further object is the provision of a method of lubrication making use of oils containing these novel ingredients.

The present invention is predicated upon the discovery that hydrocarbon oils of the classes defined above can be stabilized against the formation of acidic and/or corrosive bodies by oxidation in the presence of metals by the addition to said oils of a relatively small amount of the reaction products of cardanol ethers and halides of sulphur. The present invention is also predicated upon the discovery that novel lubricants having exceptional extreme pressure lubricating characteristics can be produced by adding to oil a sufficient quantity of these same materials. The aforesaid novel reaction products shall hereinafter be referred to as halo-sulphurized cardanol ethers, or halo-sulphurized cardanyl ethers.

As described in U. S. Patent 2,181,119, the term "cardanol" denotes a phenol having an empirical formula of  $C_{20}H_{22}O$ , and probable structural formula of  $H_2C_{14}.C_6H_4.OH$  with one unsaturated bond in the  $H_2C_{14}-$  radical, which is meta to the  $-OH$  radical. The ethers of cardanol contemplated herein are those in which the hydrogen of the  $-OH$  radical has been replaced by an organic radical, as, for example, an aromatic or an aliphatic radical, with preference given to the cardanyl alkyl ethers.

The term "cardanyl" as used herein describes that group or radical which remains on the removal of the  $-OH$  radical from cardanol, as

5



10 Making use of this term, the following structural formula represents cardanyl ethyl ether,

15



15 It is believed that sulphur mono- and di-halides react with the carbon atoms of the unsaturated bond of the  $C_{14}H_{27}$  group resulting in the formation of the sulpho-halogenated product.

20 The foregoing suggestion for the mechanism of reaction of sulphur halides and cardanol ethers is merely speculation and is not to be interpreted strictly so as to limit in any way the scope of this invention, for the halo-sulphurized cardanol ethers herein described are contemplated broadly as the reaction products of sulphur halides and cardanol ethers.

25 30 Typical halo-sulphurized cardanol ethers were prepared as follows:

(a) *Cardanyl ethyl ether-sulphur monochloride reaction product*

35 A solution of 21.4 grams of sulphur monochloride dissolved in 20 cc. of benzol is gradually added to a stirred benzol solution of cardanyl ethyl ether. The temperature is maintained at approximately 30° C. during this addition, which 40 requires about two hours. The temperature is then raised to 70° C. and maintained for a period of three hours. This is followed by water-washing until the washings are neutral. Then the 45 solution is topped under diminished pressure to 150° C. to remove solvent and to obtain the finished product. The reaction product, a brown, viscous oil, contains about 8 per cent sulphur and about 6 per cent chlorine.

50 (b) *Cardanyl ethyl ether-sulphur dichloride reaction product*

55 To a stirred benzol solution of cardanyl ethyl ether are gradually added 24.5 grams of sulphur dichloride. The temperature is maintained at approximately 30° C. during this addition which requires about one and one-half hours. The mixture is then stirred at room temperature for three hours, followed by refluxing at approximately 78° C. for three hours more. This is followed by 60 water-washing until the washings are neutral. Then, the solution is topped under diminished pressure to 175° C. to remove the solvent and to obtain the finished product. The reaction product, a brown viscous oil, contains about 6.4% sulphur and about 6.4% chlorine.

65 In preparing the finished hydrocarbon oil composition in accordance with our invention the aforesaid reaction products are intimately incorporated with or dissolved in the oil which is to be stabilized against the accelerating action of 70 reactions and against its normal tendency to corrode metal bearings, etc., and the product thus 75 obtained may then be employed for the purposes

and uses for which the unstabilized oil itself is normally employed, but with the improved results above described.

The reaction products, as produced and described, are also novel extreme pressure ingredients, and when small amounts are added to or directly dissolved in a proper hydrocarbon lubricating oil, confer upon it a greatly enhanced ability to maintain lubrication under extreme conditions of loading.

To demonstrate the effectiveness of such reaction products under actual operating conditions of an automotive engine, unblended oils and improved oils, containing the reaction products, were subjected to the Lauson engine test. The tests were carried out in a single-cylinder Lauson engine operated continuously over a time interval of 16 hours with the cooling medium held at a temperature of about 212° F. and the oil temperature held at about 280° F. The engine was operated at a speed of about 1830 R. P. M. At the end of each test the oil was tested for acidity (N. N.) and viscosity.

The following data obtained by Lauson engine tests indicate clearly the efficacy of the halo-sulphurized cardanol ethers in retarding acid formation and in retarding changes in viscosity with temperature change. This data is shown in Table I wherein the blank oil is a solvent refined oil of Saybolt Universal viscosity of 45 secs. at 210° F.

Table I

| Additive                                                      | N. N. | S. U. V.<br>@ 210° F. | Kin. visc.<br>@ 210° F. |
|---------------------------------------------------------------|-------|-----------------------|-------------------------|
| None                                                          | 3.0   | 48.40                 | 6.8                     |
| 2% cardanyl ethyl ether-sulphur monochloride reaction product | 0.7   | 46.76                 | 6.29                    |
| None                                                          | 1.7   | 46.85                 | 6.32                    |
| 2% cardanyl ethyl ether-sulphur dichloride reaction product   | 0.4   | 45.63                 | 5.83                    |

As hereinbefore mentioned, the novel reaction products contemplated herein are effective extreme pressure (E. P.) agents. Oil blends containing the typical halo-sulphurized cardanol ethers prepared above were subjected to the Almen pin test (described by Wolf and Mongey, Proc. A. P. I., 1932, pp. 118-130) and the S. A. E. test (described Anon. S. A. E. Journal 39, 23-4, 1936) with the results as shown in Table II.

Table II

| Reaction product                                  | Per cent<br>in oil | Almen pin<br>test load<br>limit,<br>pounds | S. A. E.<br>test load<br>limit,<br>pounds<br>(1,000<br>R. P. M.) |
|---------------------------------------------------|--------------------|--------------------------------------------|------------------------------------------------------------------|
| None                                              |                    | 3,000                                      | 15-20                                                            |
| Cardanyl ethyl ether-sulphur monochloride product | 10                 | 30,000+                                    | 245                                                              |
| Cardanyl ethyl ether-sulphur dichloride product   | 10                 | 30,000+                                    | -----                                                            |

The oil used in the Almen pin and S. A. E. tests was a mineral oil of 80-90 seconds Saybolt Universal viscosity at 210° F.

It will be observed that extreme pressure lubricants embodying this invention are exceptionally effective.

The proportion of the characterizing agents of this invention used in admixture with ordinary hydrocarbon lubricant oil to provide an extreme pressure lubricant may be varied. Suggested limits from about 0.25% to about 20% are those

which will convert ordinary hydrocarbon lubricants to extreme pressure lubricants capable of withstanding the conditions of use now imposed. Within this range, it is preferable with all reaction products of this class to use approximately 10 per cent. The recommended concentration of the novel reaction products of this invention for the purpose of preventing acid formation and viscosity change in temperature is

10 from about 0.25% to about 5% by weight in oil, with concentrations of the order of 2 per cent. being preferred. Thus, depending upon the oil and the results desired, the reaction products contemplated herein may be used in amounts 15 ranging from about 0.25% to about 20 per cent.

It will be understood further that the present invention is not restricted to the details of the above examples which are given merely as illustrations of this invention, but that various changes may be made in these details without departing from the true scope of this invention as defined in the appended claims.

I claim:

1. A lubricant comprising a hydrocarbon oil and a small proportion of a sulphur- and halogen-containing reaction product obtained by reaction of a cardanol ether and a sulphur halide.

2. A lubricating oil composition comprising a relatively large proportion of a lubricating oil which normally tends to rupture at the surface of contact with a bearing metal under relatively high bearing pressure and in admixture therewith a relatively small amount, sufficient to prevent such rupture, of the sulphur- and halogen-containing reaction product of a cardanol ether and a sulphur halide.

3. A lubricating oil composition comprising a relatively large proportion of a lubricating oil which tends to rupture at the surface of contact with a bearing metal under relatively high bearing pressure and in admixture therewith a relatively small amount, sufficient to prevent such rupture, of the sulphur- and chlorine-containing reaction product of a cardanol ether and sulphur monochloride.

4. A lubricating oil composition comprising a relatively large proportion of a lubricating oil which normally tends to rupture at the surface of contact with a bearing metal under relatively high bearing pressure and in admixture therewith a relatively small amount, sufficient to prevent such rupture, of the sulphur- and chlorine-containing reaction product of a cardanol ether and sulphur dichloride.

5. A lubricating oil composition comprising a relatively large proportion of a lubricating oil which normally tends to rupture at the surface of contact with a bearing metal under relatively high bearing pressure and in admixture therewith a relatively small amount, sufficient to prevent such rupture, of the sulphur- and chlorine-containing reaction product of a cardanyl alkyl ether and a sulphur halide.

6. A lubricating oil composition comprising a relatively large proportion of a lubricating oil which normally tends to rupture at the surface of contact with a bearing metal under relatively high bearing pressure and in admixture therewith a relatively small amount, sufficient to prevent such rupture, of the sulphur- and chlorine-containing reaction product of a cardanyl alkyl ether and sulphur monochloride.

7. A lubricating oil composition comprising a relatively large proportion of a lubricating oil

which normally tends to rupture at the surface of contact with a bearing metal under relatively high bearing pressure and in admixture therewith a relatively small amount, sufficient to prevent such rupture, of the sulphur- and chlorine-containing reaction product of a cardanyl alkyl ether and sulphur dichloride.

8. A lubricating oil composition comprising a relatively large proportion of a lubricating oil which normally tends to rupture at the surface of contact with a bearing metal under relatively high bearing pressure and in admixture therewith a relatively small amount, sufficient to prevent such rupture, of the sulphur- and halogen-containing reaction product of cardanyl ethyl ether and a sulphur halide.

9. A lubricating oil composition comprising a relatively large proportion of a lubricating oil which normally tends to rupture at the surface of contact with a bearing metal under relatively high pressure and in admixture therewith a relatively small amount, sufficient to prevent such rupture, of the sulphur- and chlorine-containing reaction product of cardanyl ethyl ether and sulphur monochloride.

10. A lubricating oil composition comprising a relatively large proportion of a lubricating oil which normally tends to rupture at the surface of contact with a bearing metal under relatively high pressure and in admixture therewith a relatively small amount, sufficient to prevent such rupture, of the sulphur- and chlorine-containing

reaction product of cardanyl ethyl ether and sulphur dichloride.

11. The method of lubricating relatively moving metal parts wherein unit bearing pressures of high magnitude are developed, which comprises applying to the area of contact between said parts a mixture of viscous petroleum oil and a small proportion, sufficient to increase the load carrying capacity of the mixture, of the sulphur- and halogen-containing reaction product of a cardanol ether and a sulphur halide.

12. A lubricating oil composition comprising a relatively large proportion of a lubricating oil of the type normally tending to deteriorate by oxidation under normal conditions of use involving the accelerating action of metals and in intimate admixture therewith a relatively small proportion, sufficient to inhibit such deterioration, of the sulphur- and chlorine-containing reaction product of a cardanol ether and a sulphur halide, said composition being further characterized by a relatively high stability toward viscosity change with temperature change under normal conditions of use.

13. A lubricant comprising a hydrocarbon oil and a small proportion of a sulphur- and halogen-containing reaction product obtained by reaction of a cardanol ether and a sulphur halide, said reaction product being present in an amount of from about 0.25% to about 20 per cent.

FERDINAND P. OTTO.